

(No Model.)

T. J. TRESIDDER.  
MANUFACTURE OF ARMOR PLATES.

No. 475,364.

Patented May 24, 1892.

Fig. 1.



Fig. 2.



Fig. 4.



Fig. 5.



Fig. 3.



Fig. 7.



Witnesses.

W. Washington Miller  
C. M. Brooke.

Inventor

Tolmie John Tresidder,  
By his Attorneys,  
Baldwin, Davidson & Night

# UNITED STATES PATENT OFFICE.

TOLMIE JOHN TRESIDDER, OF SHEFFIELD, ENGLAND.

## MANUFACTURE OF ARMOR-PLATES.

SPECIFICATION forming part of Letters Patent No. 475,364, dated May 24, 1892.

Application filed September 8, 1891. Serial No. 406,097. (No model.) Patented in France September 3, 1891, No. 215,886, and in Italy September 30, 1891, No. 30,334.

*To all whom it may concern:*

Be it known that I, TOLMIE JOHN TRESIDDER, a subject of the Queen of Great Britain, now residing at the Atlas Steel Works, Sheffield, in the county of York, England, have invented certain new and useful Improvements in the Manufacture of Armor-Plates, (for which I have obtained the following patents, viz: French Patent No. 215,886, dated 5 September 3, 1891, and Italian Patent No. 30,334, dated September 30, 1891,) of which the following is a specification.

When a water bath is employed in hardening pieces of steel in large bulk unsatisfactory 15 results are obtained mainly on account of the formation of a steam envelope around the immersed article, which envelope being continually broken and reformed during the early 20 stages of quenching only allows the heat to be abstracted spasmodically instead of with the uniformity which is the first requisite for a successful result. The superior action of an oil bath is due not to the chemical composition of oil, but to the absence of the steam 25 envelope. Where glycerine or any substance tending to raise the boiling-point is added to a water bath, the result is improved for a similar reason.

According to my present invention I manufacture 30 armor-plates, giving to them the requisite shape, strength, hardness, and tenacity by a process which does away with the formation of a steam-envelope.

According to my invention I may use water 35 or similar chilling fluid without encountering the objectionable features above referred to. I preferably use water; but I do not limit myself to the use of water alone, as my process has the contingent advantage of allowing any 40 fluid, gas, or vapor to be uniformly applied to one side only of an armor-plate or similar article, which would not be possible by immersion in a bath unless the surface to be treated happened to be perfectly flat.

It is well known that in the manufacture 45 of armor-plates serious difficulties have been encountered owing to the warping of the plate by the hardening or tempering process, which 50 distorts it from the desired shape or designer's templet. When armor-plates are thus warped

or distorted, it is very difficult to get them into proper shape; but according to my process this difficulty or objection is done away with.

In carrying out my invention I preferably use apparatus such as shown in the accompanying drawings, in which—

Figure 1 is a plan view of a douche or spraying apparatus which I may employ. Fig. 2 is a side view of my apparatus for use on a plate intended to be finished flat or slightly curved. Fig. 3 is a side view of a modification thereof in use with a plate of considerable curvature. Fig. 4 shows a guard to prevent the too-rapid cooling of the corners of plates. Fig. 5 is a guard of different form to 65 protect the edges. Fig. 6 shows a perspective view of a portion of a plate provided with corner and edge protecting guards. Fig. 7 is a section of a portion of the end of the plate. Fig. 8 is a section of a perforated water-pipe. 70

Referring now to the details of my drawings by letters, *a a a a* (see Fig. 1) are four-inch quarter-bends with flanges.

*b* is a four-inch straight pipe.

*c* is a four-inch pipe with two four-inch connections *d d* from the water-service. To the pipes *b c* are connected two four-inch pipes *e e*, cast with numerous teats for one-inch screw connections, in which are screwed a series of one-inch cross-pipes *f f f*, having the 80 long unions *g g*. These pipes are full of one-eighth-inch perforations on the under side, drilled at various angles to spread the jets of water. Douches of different sizes should be provided—some flat, as above, and others 85 more or less curved.

*b<sup>2</sup>* is an armor-plate, bent concave to finish flat.

In Fig. 2, *a<sup>2</sup> a<sup>2</sup>* is the douche above described. *c<sup>2</sup> c<sup>2</sup> c<sup>2</sup>* is a tray adapted to hold water up against the back of the plates. *d<sup>2</sup> d<sup>2</sup>* are cast-iron pyramids on which the plate rests. *e<sup>2</sup> e<sup>2</sup>* indicate water overflowing the edges of the tray and running to waste. *X* is one of the water-inlets.

In Fig. 3, *a<sup>3</sup> a<sup>3</sup>* is the upper douche for hardening a curved plate. *b<sup>3</sup> b<sup>3</sup>* is the lower douche for moderating the warp, and *c<sup>3</sup> c<sup>3</sup> c<sup>3</sup>* are the water-inlets, both douches being substantially like that shown in Fig. 1, but 100

curved to suit the curved armor-plate, (indicated by  $d^3 d^3$ ).  $e^3 e^3$  are the keyways in edges temporarily filled up. The full line shows the curve of the false templet and the dotted line that of the designer's templet.

Fig. 4 shows a shoe with a clamping-screw  $s$  to attach to the corners of the plate when required to prevent them from too rapidly cooling. The top  $a^4$  rests on the top of the plate and the clamping-screw bites on the under surface. It is cast-iron, about one inch thick and beveled to one-fourth of an inch at the edge  $b^4$ , which is curved, as shown.

Fig. 5 shows an edge-guard with clamping-screws  $s$  to attach to the plates when required to check the chilling of their edges. This will be straight or curved, as required, The upper flange rests on the top of the plate and the clamping-screws bite on the under surface.

By my process, as will be further explained hereinafter, I obtain, first, intense hardness and tenacity in the faces of compound armor-plates; (steel faced with iron backs;) second, intense hardness and tenacity in the faces of compound steel armor-plates, (all steel with or without nickel, &c., with high carbon faces and mild backs, whether built up or made originally homogeneous and subsequently "converted" on one side,) and, third, increased tenacity and toughness, such as has hitherto been obtained by oil-hardening followed by annealing in homogeneous steel armor-plates, whether containing chrome, nickel, or other such ingredients or not. The injurious and commonly fatal internal strains induced in a large mass of steel by quenching it in a water bath are entirely avoided by my process, which at the same time retains all the valuable properties inherent to water-quenching.

Before describing my method of using the apparatus I will state that repeated experiments have shown me that the warping produced by quenching a straight plate nine or ten inches thick from one side only is of a uniform convexity toward the quenched side, and that the amount of convexity is about three-eighths of an inch in a distance of four feet; also, that the warping of a steel-faced compound plate of the same thickness quenched from both sides is similar in nature, but less in extent, being at the rate of about one-fourth of an inch in a distance of four feet. Homogeneous steel plates equally quenched from both sides after being uniformly heated have no tendency to warp. Experiment has also shown me that by bending a flat plate till it is concave on the side to be hardened to an extent determined in the manner above specified, its flatness will be restored by the warp due to quenching. Thus plates to be treated by this process must be originally bent with less convexity on the hard side than ultimately required, and to do this properly I provide false templets, to which the plates are to be bent. The proper form for these false templets can

be arrived at approximately by applying one of the corrections given above and with accuracy after a few trials with the particular kind of plate to be treated. Thinner plates warp more than thicker ones. A plate four inches thick shows a convexity of one-half an inch in four feet when hardened on one side only. This being understood, I will proceed to describe my process of treating various plates, as follows:

First. If the plate be treated is a compound plate (steel face and iron back) to finish approximately flat, (as belt-plates,) I make it and machine it in the usual way, except that I use false templets to which to bend it. These false templets are constructed from the designer's templets. When the plate is finished as far as regards all machine-work to the steel portion, all holes (if there be any such, as those tapped in the top edges of belt-plates for the deck attachment) in the steel are plugged with flush wrought-iron screw-plugs arranged so as to be withdrawn with facility. Similarly, any keyways in the edges, if in the steel portion, are fitted with temporary keys  $k$ . The plate  $b^2$  is then carefully heated in a furnace to a "hardening heat," which will of course vary with the nature of the steel. Ordinarily a moderate red heat will suffice. When hot enough, it is taken from the furnace and deposited steel side up on four supports  $d^2$  in a large flat tray  $c^2$  (see Fig. 2) in such a way that the edge of the tray is everywhere a little higher than the bottom of the plate. The douche  $a^2$  is then brought up and supported a little above the plate, and the water, which is preferably at a high pressure—say eighty pounds to the square inch—is turned on. At first the water quenches the steel side only; but in a few moments the tray becomes full and forms a bath for the lower iron side. The object of this is to reduce the warping of the plate, which it does by about one-half. It also tends to assist the chilling action of the douche above, but the soft iron on which it acts is not affected. If the utmost possible degree of hardness is desired, the douching is continued till the plate is cold; but I sometimes stop the water after all redness has disappeared, throw on the plate some scraps of soft alloy, and turn on the water again as soon as these scraps show signs of melting. In this way by using alloys of suitable melting-points the plate can be tempered with great nicety to any required degree. When the plate is cold, it will be found to have its proper finished shape if the false templets have been correctly made and worked to. The temporary plugs and keys (if any) can be withdrawn and the bolt-holes drilled and tapped in the back to complete the plate. No correction whatever of the edges should be required; but if it proves necessary it will be so small as to be readily corrected by grinding with an emery-wheel. In order to prevent too great rapidity of cooling at the corners of the plate, I sometimes

attach thereto iron shoes, Fig. 4, which modify the chilling action of the water at those parts. In special cases the edges of the plate also may be protected in a similar manner by the guards shown at Fig. 5, even to the extent of keeping them soft enough to be machined.

Second. If the plate to be hardened is a compound plate (steel face and iron back) to be finished with considerable curvature, (as a turret or conning-tower plate,) I proceed exactly as described above, except that instead of a tray I use a second douching apparatus to cool the under side of the plate, Fig. 3. This acts upward; but it must be remembered in all cases that the douche which is to harden the plate is at its best advantage when acting directly downward. In Fig. 3 the full lines show the curve of the metal before hardening, while the dotted lines show the curve when the plate is cooled.

Third. If the plate to be treated is a compound steel plate in which the back is of so mild a nature as to undergo water-quenching without losing toughness, the double douche, as described, for a curved compound plate may be used; but if it is undesirable to quench the back, then the downward douche on the face only, without any tray to hold the water up against the back, is to be preferred. In some cases I use the double douche with water above the plate and air or wet air below.

Fourth. If the plate to be treated is a homogeneous steel plate requiring toughness throughout rather than a hard face, either the double douche or the single douche with tray will be efficient. In a case of this kind I prefer to use a double douche of wet air applied in the same way as the water.

As regards the water-pressure to be used I prefer a high pressure—say eighty pounds to the square inch; but this depends greatly upon the area of the surface to be treated. In any case there must be sufficient volume of water to cause a brisk flow from all the apertures of the douching apparatus. For the air or wet-air quenching a pressure of about ten pounds to the inch will suffice.

In cases where it is not desirable to let the water run to waste, or where the douching apparatus is employed with special fluids which are of value, arrangements can easily be made for catching the fluid as it falls from the plate and conveying it to a tank to be pumped and used over again.

The action of the water-douche on high-carbon steel is, as might be expected, to produce intense hardness. As the carbon is lower the hardening becomes less marked;

but an appreciable hardening or stiffening effect is produced with steels containing as little as two-tenths of one per cent. of carbon. In such a case the effect of the treatment resembles that obtained by hardening a steel of somewhat higher carbon in oil at, say,  $1,600^{\circ}$  Fahrenheit, and then annealing at, say,  $900^{\circ}$  Fahrenheit. The wet air has a milder action (on large masses,) about that of oil-hardening at  $1,300^{\circ}$  Fahrenheit and annealing at  $1,200^{\circ}$  Fahrenheit. Dry air, especially hot dry air, has the mildest effect of all; but the uniform distribution of the cooling action peculiar to this invention always results in improving the steel.

By the treatment above set forth I am enabled to readily produce tempered and hardened plates of the right shape, notwithstanding the warping caused by the process of hardening or tempering as usually carried out, and should any of the plates fail to fit it will be found that they are so little out of their designed shaped that they can be readily fitted by grinding.

I claim as my invention—

1. The herein - described method for the manufacture of armor-plates, which consists in making and machining the plate, plugging the holes and keyways, protecting the edges and corners by shoes or guards, heating the plate to a hardening heat, and then subjecting it to sprays of a chilling-fluid acting downwardly upon its front or shot-receiving side.

2. The herein - described method for the manufacture of armor-plates, which consists in making and finishing the plate to a shape indicated by a false templet different from the designer's templet, heating the plate to a hardening heat, and subjecting the steel or shot-receiving side of the plate to sprays of a chilling fluid to harden said shot-receiving side and bend the plate to the form required for use.

3. The herein - described method for the manufacture of armor-plates, which consists in forming a plate to a shape indicated by a false templet different from the designer's templet, heating the plate to a hardening heat, and simultaneously subjecting both the shot-receiving side and the rear side of the plate to sprays of a chilling fluid to harden and bend it to the form required for use.

TOLMIE JOHN TRESIDDER.

Witnesses:

C. B. HOBBS,

HAROLD P. BURDEKIN,

Clerks to Messrs. Burdekin & Co., Solrs.,  
Sheffield, England.